



US008470505B2

(12) **United States Patent**  
**Yu et al.**

(10) **Patent No.:** **US 8,470,505 B2**  
(45) **Date of Patent:** **Jun. 25, 2013**

(54) **IMAGING MEMBERS HAVING IMPROVED IMAGING LAYERS**

(75) Inventors: **Robert C. U. Yu**, Webster, NY (US); **Yuhua Tong**, Webster, NY (US)

(73) Assignee: **Xerox Corporation**, Norwalk, CT (US)

(\*) Notice: Subject to any disclaimer, the term of this patent is extended or adjusted under 35 U.S.C. 154(b) by 274 days.

(21) Appl. No.: **12/813,240**

(22) Filed: **Jun. 10, 2010**

(65) **Prior Publication Data**

US 2011/0305981 A1 Dec. 15, 2011

(51) **Int. Cl.**  
**G03G 5/04** (2006.01)

(52) **U.S. Cl.**  
USPC ..... **430/59.6; 430/58.8; 399/159**

(58) **Field of Classification Search**  
USPC ..... **430/58.8, 59.6; 399/159**  
See application file for complete search history.

(56) **References Cited**

U.S. PATENT DOCUMENTS

|             |         |                  |
|-------------|---------|------------------|
| 3,121,006 A | 2/1964  | Middleton et al. |
| 3,820,989 A | 6/1974  | Rule et al.      |
| 3,837,851 A | 9/1974  | Shattuck et al.  |
| 3,895,944 A | 7/1975  | Wiedemann et al. |
| 4,150,987 A | 4/1979  | Anderson et al.  |
| 4,245,021 A | 1/1981  | Kazami et al.    |
| 4,256,821 A | 3/1981  | Enomoto et al.   |
| 4,265,990 A | 5/1981  | Stolka et al.    |
| 4,278,746 A | 7/1981  | Goto et al.      |
| 4,286,033 A | 8/1981  | Neyhart et al.   |
| 4,297,426 A | 10/1981 | Sakai et al.     |
| 4,315,982 A | 2/1982  | Ishikawa et al.  |

|             |         |                      |
|-------------|---------|----------------------|
| 4,338,387 A | 7/1982  | Hewitt               |
| 4,338,388 A | 7/1982  | Sakai et al.         |
| 4,385,106 A | 5/1983  | Sakai                |
| 4,387,147 A | 6/1983  | Sakai                |
| 4,399,207 A | 8/1983  | Sakai et al.         |
| 4,399,208 A | 8/1983  | Takasu et al.        |
| 4,587,189 A | 5/1986  | Hor et al.           |
| 4,664,995 A | 5/1987  | Horgan et al.        |
| 4,988,597 A | 1/1991  | Spiewak et al.       |
| 5,215,839 A | 6/1993  | Yu                   |
| 5,244,762 A | 9/1993  | Spiewak et al.       |
| 5,660,961 A | 8/1997  | Yu                   |
| 5,697,024 A | 12/1997 | Mishra               |
| 5,703,487 A | 12/1997 | Mishra               |
| 5,756,245 A | 5/1998  | Esteghamatian et al. |
| 5,958,638 A | 9/1999  | Katayama et al.      |
| 6,008,653 A | 12/1999 | Popovic et al.       |
| 6,119,536 A | 9/2000  | Popovic et al.       |
| 6,124,514 A | 9/2000  | Emmrich et al.       |
| 6,150,824 A | 11/2000 | Mishra et al.        |

(Continued)

FOREIGN PATENT DOCUMENTS

JP 2000-162810 \* 6/2000

OTHER PUBLICATIONS

Translation of JP 2000-162810 published Jun. 2000.\*

Primary Examiner — Peter Vajda

(74) Attorney, Agent, or Firm — Pillsbury Winthrop Shaw Pittman LLP

(57) **ABSTRACT**

The presently disclosed embodiments are directed to imaging members used in electrostatography. More particularly, the embodiments pertain to electrophotographic imaging members which have imaging layer(s) formulated to comprise of a novel A-B diblock copolymer binder consisting of two segmental blocks of a bisphenol polycarbonate and a phthalic acid which provides chemical vapor contaminant resistive property. The present embodiments provide superior copy printout quality.

**19 Claims, 4 Drawing Sheets**



**US 8,470,505 B2**

Page 2

---

U.S. PATENT DOCUMENTS

|              |         |                 |                   |        |                              |
|--------------|---------|-----------------|-------------------|--------|------------------------------|
| 6,214,514 B1 | 4/2001  | Evans et al.    | 7,033,714 B2      | 4/2006 | Horgan et al.                |
| 6,326,111 B1 | 12/2001 | Chambers et al. | 7,413,835 B2      | 8/2008 | Lin et al.                   |
| 6,756,169 B2 | 6/2004  | Lin et al.      | 7,592,111 B2      | 9/2009 | Yu et al.                    |
| 6,933,089 B2 | 8/2005  | Horgan et al.   | 2005/0136349 A1 * | 6/2005 | Mishra et al. .... 430/58.05 |
| 7,018,756 B2 | 3/2006  | Pai et al.      | 2007/0099101 A1 * | 5/2007 | Horgan et al. .... 430/58.75 |

\* cited by examiner



**FIG. 1**  
PRIORITY ART



FIG. 2



FIG. 3



FIG. 4



FIG. 5



FIG. 6

## IMAGING MEMBERS HAVING IMPROVED IMAGING LAYERS

### BACKGROUND

The presently disclosed embodiments are directed to imaging members used in electrostatography. More particularly, the embodiments are pertaining to electrophotographic imaging member which has improved imaging layer(s) formulated to consist of a novel polycarbonate binder that has chemical vapor contaminant resistive property to preserve copy print-out quality. The present disclosure relates to all types of electrophotographic imaging members used in electrophotography.

In electrostatographic reproducing apparatuses, including digital, image on image, and contact electrostatic printing apparatuses, a light image of an original to be copied is typically recorded in the form of an electrostatic latent image upon a photosensitive member and the latent image is subsequently rendered visible by the application of electroscopic thermoplastic resin particles and pigment particles, or toner. Flexible electrostatographic imaging members are well known in the art. Typical electrostatographic imaging members include, for example: (1) electrophotographic imaging members (photoreceptors) commonly utilized in electrophotographic (xerographic) processing systems; (2) electroreceptors such as ionographic imaging members for electrographic imaging systems; and (3) intermediate toner image transfer members such as an intermediate toner image transferring belt which is used to remove the toner images from a photoreceptor surface and then transfer the very images onto a receiving paper. All the electrostatographic imaging members are prepared in either flexible belt form or rigid drum configuration. For typical flexible electrophotographic imaging member belt, it comprises a charge transport layer, a charge generating layer, and optional layers on one side of a supporting substrate layer and does also include an anti back coating on the opposite side of the substrate to imaging member flatness. For a typical flexible electrographic imaging member belt, it does, however, have a more simple material structure; it includes a dielectric imaging layer on one side of a supporting substrate and an anti-curl back coating on the opposite side of the substrate to render flatness. Alternatively, the electrostatographic imaging members can also be a rigid member, such as those utilizing a rigid substrate support drum. For these drum imaging members, having a thick rigid cylindrical supporting substrate bearing the imaging layer(s), there is no exhibition of the curl-up problem, and thus, there is no need for an anticurl back coating layer.

The flexible electrostatographic imaging members may be seamless or seamed belts. Seamed belts are usually formed by cutting a rectangular sheet from a web, overlapping opposite ends, and welding the overlapped ends together to form a welded seam.

Although the scope of the present embodiments covers the preparation of all types of electrostatographic imaging members in flexible belt design or rigid drum configuration, however, for reason of simplicity, the discussion hereinafter will focus and be represented only on flexible electrophotographic imaging member belts.

One type of flexible composite photoconductive layer used in xerography is illustrated in U.S. Pat. No. 4,265,990 which describes a photosensitive imaging member having at least two electrically operative layers. One layer comprises a photoconductive layer which is capable of photogenerating holes and injecting the photogenerated holes into a contiguous charge transport layer. Generally, the two electrically opera-

tive layers are supported on a conductive layer support substrate, with the photoconductive layer being sandwiched between a contiguous charge transport layer and the supporting conductive layer. In this negatively charged imaging member, the charge transport layer is therefore the top outermost exposed layer. In the alternative imaging member design, the charge transport layer is, however, sandwiched between the supporting electrode and a photoconductive layer. Since the typical flexible electrophotographic imaging members exhibit undesirable upward imaging member curling-up after completion of the electrically operative layers, the application of an anticurl back coating onto the backside of the support substrate is necessary to provide the appropriate imaging members with desirable flatness.

15 The flexible photosensitive members having at least two electrically operative layers, as disclosed above, provide excellent electrostatic latent images when charged in the dark with a uniform negative electrostatic charge, exposed to a light image and thereafter developed with finely divided electroscopic marking particles. The resulting toner image is usually transferred to a suitable receiving member such as paper or to an intermediate transfer member which thereafter transfers the image to a receiving member such as paper.

20 In the case where the charge generating layer is sandwiched between the top outermost exposed charge transport layer and the electrically conducting layer, the outer surface of the charge transport layer is charged negatively and the conductive layer is charged positively. The charge generating layer then should be capable of generating electron hole pair 25 when exposed image wise and inject only the holes through the charge transport layer. In the alternate case when the charge transport layer is sandwiched between the charge generating layer and the conductive layer, the outer surface of the charge generating layer is charged positively while conductive layer is charged negatively and the holes are injected through from the charge generating layer to the charge transport layer. The charge transport layer should be able to transport the holes with as little trapping of charge as possible. In 30 flexible imaging member belt such as photoreceptor, the charge conductive layer may be a thin coating of metal on a flexible substrate support layer.

25 As more advanced, higher speed electrophotographic copiers, duplicators and printers were developed, however, degradation of image quality was encountered during extended cycling. The complex, highly sophisticated duplicating and printing systems operating at very high speeds have placed stringent requirements including narrow operating limits on photoreceptors. For example, the numerous layers used in many modern photoconductive imaging members should be 35 highly flexible, adhere well to adjacent layers, and exhibit predictable electrical characteristics within narrow operating limits to provide excellent toner images over many thousands of cycles. Typically, negatively charged multilayered flexible photoreceptor that has been employed as a belt in electrophotographic imaging systems comprises a flexible substrate, a conductive layer, an optional blocking layer, an optional adhesive layer, a charge generating layer, a charge transport layer and a conductive ground strip layer adjacent to one edge of the imaging layers. In such a photoreceptor, it does usually 40 further comprise an anticurl back coating layer on the side of the substrate opposite the side carrying the conductive layer, support layer, blocking layer, adhesive layer, charge generating layer, charge transport layer, and other layers to effect for curl control.

45 55 60 65 Since the charge transport layer in a negatively charged imaging member is the top outermost exposed layer, it is constantly subjected to chemical vapor contaminants expo-

3

sure/interaction during electrophotographic imaging process in the field to negatively impact function. For example, exposure to the vapor amine species (from ammonia) emitted from common house cleaning agents have been seen to interact with the imaging member charge transport layer, causing material degradation to promote pre-mature onset of charge transport layer cracking and exacerbation of wear failure which severely cut short the functional life of the imaging member. In one particular instant, amine vapor impact on copy printout quality degradation has recently been seen when pre-printed papers (papers having pre-printed images which employed amine agents catalyzed UV cured ink) are used by customers for subsequent addition of xerographic images over the pre-printed paper blank spaces; that is the accumulation of amine residues deposition onto the imaging member charge transport layer surface, after repeatedly making contact with receiving papers during xerographic imaging process, is found to cause ghosting image defects print-out in the output copies. Since ghosting image defects in the output copies are unacceptable print quality failures, so it does require frequent costly imaging member replacement in the field. With all these issues and failures described above, therefore there is an urgent need to resolve these issues and extend the service life of the imaging member in the field. In particu-

4

## SUMMARY

According to aspects illustrated herein, there is an imaging member comprising: a flexible substrate; a charge generating layer disposed on the substrate; and at least one charge transport layer disposed on the charge generating layer, wherein the charge transport layer comprises a charge transport component molecularly dispersed in a polycarbonate binder, the polycarbonate binder being an A-B diblock copolymer comprising two segmental blocks of a bisphenol A polycarbonate ( $C_{16}H_{14}O_3$ ) and a phthalic acid capable of providing protection against amine species contaminants.

15 Another embodiment provides an imaging member comprising: a substrate; a charge generating layer disposed on the substrate; a bottom charge transport layer disposed on the charge generating layer; and a top exposed charge transport layer disposed on the bottom charge transport layer, wherein  
20 both the bottom and the top exposed charge transport layers comprise N,N'-diphenyl-N,N'-bis(3-methylphenyl)-1,1-bi-phenyl-4,4'-diamine molecularly dispersed in a polycarbonate binder, the polycarbonate binder having a formula selected from the group consisting of



lar, by the formulation of a charge transport layer that is resistive to amine specific effect to resolve the current pre-printed paper ghosting image defects print out problem.

Conventional photoreceptors are disclosed in the following patents, a number of which describe the presence of light scattering particles in the undercoat layers: U.S. Pat. Nos.

wherein z represents the number of bisphenol A repeating units in block A and is from about 9 to about 18, y represents the number of repeating phthalic acid in block B and is from about 1 to about 2, and n represents the degree of polymerization of di-block copolymer and is from about 20 to about 80,



5,660,961; 5,215,839; and 5,958,638. The term "photoreceptor" or "photoconductor" is generally used interchangeably with the terms "imaging member." The term "electrostatographic" includes "electrophotographic" and "xerographic." The terms "charge transport molecule" are generally used interchangeably with the terms "hole transport molecule."

In U.S. Pat. No. 7,413,835, there is disclosed an electro-photographic imaging member having a thermoplastic charge transport layer, a polycarbonate polymer binder, a particulate dispersion, and a high boiler compatible liquid. The disclosed charge transport layer exhibits enhanced wear resistance, excellent photoelectrical properties, and good print quality.

In U.S. Pat. No. 7,592,111, there is disclosed an imaging member formulated with a liquid carbonate. The imaging electrostatographic member exhibits improved service life.

wherein z represents the number of bisphenol A repeating units in block A and is from about 9 to about 18, y represents the number of repeating phthalic acid in block B and is from about 1 to about 2, and n represents the degree of polymerization of di-block copolymer and is from about 20 to about 80, and mixtures thereof.

Yet another embodiment, there is an image forming apparatus for forming images on a recording medium comprising:  
a) imaging member having a charge retentive-surface for receiving an electrostatic latent image thereon, wherein the imaging member comprises a flexible substrate; a charge generating layer disposed on the substrate; and at least one charge transport layer disposed on the charge generating layer, wherein the charge transport layer comprises a charge transport component molecularly dispersed in a polycarbon-

ate binder, the polycarbonate binder being an A-B di-block copolymer comprising two segmental blocks of a Bisphenol A polycarbonate ( $C_{16}H_{14}O_3$ ) and a phthalic acid; b) a development component for applying a developer material to the charge-retentive surface to develop the electrostatic latent image to form a developed image on the charge-retentive surface; c) a transfer component for transferring the developed image from the charge-retentive surface to a copy substrate; and d) a fusing component for fusing the developed image to the copy substrate.

#### BRIEF DESCRIPTION OF THE DRAWINGS

For a better understanding of the details of present disclosure, reference may be had to the accompanying figures.

FIG. 1 is a cross-sectional view of a conventional flexible multilayered electrophotographic imaging member;

FIG. 2 is a cross-sectional view of a flexible multilayered electrophotographic imaging member having a single charge transport layer according to the present embodiments;

FIG. 3 is a cross-sectional view of a flexible multilayered electrophotographic imaging member having dual charge transport layers according to the present embodiments;

FIG. 4 is a cross-sectional view of a flexible multilayered electrophotographic imaging member having triple charge transport layers according to an embodiment of the present disclosure.

#### DETAILED DESCRIPTION OF THE DRAWINGS

In the following description, reference is made to the accompanying drawings, which form a part hereof and which illustrate several embodiments. It is understood that other embodiments may be utilized and structural and operational changes may be made without departure from the scope of the present embodiments.

According to aspects illustrated herein, there is provided a flexible imaging member comprising a flexible substrate, a charge generating layer disposed on the substrate, and at least one charge transport layer disposed on the charge generating layer, wherein the charge transport layer comprises a charge transport compound of N,N'-diphenyl-N,N'-bis(3-methylphenyl)-1,1-biphenyl-4,4'-diamine and a polycarbonate binder which is an A-B diblock copolymer derived from a bisphenol polycarbonate modified to contain about 10 mole percent of a phthalic acid containing block at the terminal of the main polycarbonate chain.

In the example of one specific electrophotographic imaging member, the charge transport layer of the present disclosure is formulated to comprise a charge transport component molecularly dispersed in a novel A-B diblock copolymer binder; the copolymer binder is created by modifying the bisphenol A polycarbonate poly(4,4'-isopropylidene diphenyl carbonate) to include a phthalic acid containing segmental block B at the terminal of the bisphenol A polycarbonate backbone. Therefore, the A-B di-block copolymer is consisting of a bisphenol A polycarbonate segment block A and a phthalic acid containing segment block B, having a general molecular structure shown in Formula (I) below:



FIG. 5 is a cross-sectional view of a flexible multilayered electrophotographic imaging member having multiple charge transport layers according to an embodiment of the present disclosure; and

FIG. 6 is a cross-sectional view of a flexible multilayered electrophotographic imaging member having a single charge generating/transporting layer according to the present embodiments.

In another electrophotographic imaging member example, the charge transport layer of this disclosure is also formulated 45 to comprise a charge transport component molecularly dispersed in a likewise film forming A-B diblock copolymer binder consisting of a bisphenol A polycarbonate poly(4,4'-isopropylidene diphenyl carbonate) block A and a phthalic acid containing segmental block B at the terminal of bisphenol 50 A polycarbonate back bone. The likewise A-B diblock copolymer of the bisphenol A polycarbonate does have a general molecular structure shown in the following Formula (II):



In the above formulas, z represents the number of bisphenol A repeating units in block A of from about 9 to about 18, y is number of repeating phthalic acid block B of from about 1 to about 2, and n is the degree of polymerization. The degree of polymerization, n, is between about 20 and about 80 of the diblock copolymer having molecular weight between about 100,000 and about 200,000.

A typical conventional negatively charged flexible electrophotographic imaging member of prior art is illustrated in FIG. 1. The substrate 10 has an optional conductive layer 12. An optional hole blocking layer 14 disposed onto the conductive layer 12 is coated over with an optional adhesive layer 16. The charge generating layer 18 is located between the adhesive layer 16 and the charge transport layer 20. An optional ground strip layer 19 operatively connects the charge generating layer 18 and the charge transport layer 20 to the conductive ground plane 12, and an optional overcoat layer 32 is applied over the charge transport layer 20. An anti-curl backing layer 1 is applied to the side of the substrate 10 opposite from the electrically active layers to render imaging member flatness.

The layers of the imaging member include, for example, an optional ground strip layer 19 that is applied to one edge of the imaging member to promote electrical continuity with the conductive ground plane 12 through the hole blocking layer 14. The conductive ground plane 12, which is typically a thin metallic layer, for example a 10 nanometer thick titanium coating, may be deposited over the substrate 10 by vacuum deposition or sputtering process. The other layers 14, 16, 18, 20 and 43 are to be separately and sequentially deposited, onto to the surface of conductive ground plane 12 of substrate 10 respectively, as wet coating layer of solutions comprising a solvent, with each layer being dried before deposition of the next subsequent one. An anticurl back coating layer 1 may then be formed on the backside of the support substrate 1. The anticurl back coating 1 is also solution coated, but is applied to the back side (the side opposite to all the other layers) of substrate 1, to render imaging member flatness.

#### The Substrate

The imaging member support substrate 10 may be opaque or substantially transparent, and may comprise any suitable organic or inorganic material having the requisite mechanical properties. The entire substrate can comprise the same material as that in the electrically conductive surface, or the electrically conductive surface can be merely a coating on the substrate. Any suitable electrically conductive material can be employed. Typical electrically conductive materials include copper, brass, nickel, zinc, chromium, stainless steel, conductive plastics and rubbers, aluminum, semitransparent aluminum, steel, cadmium, silver, gold, zirconium, niobium, tantalum, vanadium, hafnium, titanium, nickel, chromium, tungsten, molybdenum, paper rendered conductive by the inclusion of a suitable material therein or through conditioning in a humid atmosphere to ensure the presence of sufficient water content to render the material conductive, indium, tin, metal oxides, including tin oxide and indium tin oxide, and the like. It could be single metallic compound or dual layers of different metals and or oxides.

The support substrate 10 can also be formulated entirely of an electrically conductive material, or it can be an insulating material including inorganic or organic polymeric materials, such as, MYLAR, a commercially available biaxially oriented polyethylene terephthalate from DuPont, or polyethylene naphthalate (PEN) available as KALEDEX 2000, with a ground plane layer comprising a conductive titanium or titanium/zirconium coating, otherwise a layer of an organic or inorganic material having a semiconductive surface layer,

such as indium tin oxide, aluminum, titanium, and the like, or exclusively be made up of a conductive material such as, aluminum, chromium, nickel, brass, other metals and the like. The thickness of the support substrate depends on numerous factors, including mechanical performance and economic considerations. The substrate may have a number of many different configurations, such as, for example, a plate, a drum, a scroll, an endless flexible belt, and the like. In one embodiment, the substrate is in the form of a seamed flexible belt.

The thickness of the support substrate 10 depends on numerous factors, including flexibility, mechanical performance, and economic considerations. The thickness of the support substrate may range from about 50 micrometers to about 3,000 micrometers. In embodiments of flexible imaging member belt preparation, the thickness of substrate used is from about 50 micrometers to about 200 micrometers for achieving optimum flexibility and to effect tolerable induced imaging member belt surface bending stress/strain when a belt is cycled around small diameter rollers in a machine belt support module, for example, the 19 millimeter diameter rollers.

An exemplary functioning support substrate 10 is not soluble in any of the solvents used in each coating layer solution, has good optical transparency, and is thermally stable up to a high temperature of at least 150° C. A typical support substrate 10 used for imaging member fabrication has a thermal contraction coefficient ranging from about  $1 \times 10^{-5}/^{\circ}\text{C}$ . to about  $3 \times 10^{-5}/^{\circ}\text{C}$ . and a Young's Modulus of between about  $5 \times 10^{-5}$  psi ( $3.5 \times 10^{-4}$  Kg/cm<sup>2</sup>) and about  $7 \times 10^{-5}$  psi ( $4.9 \times 10^{-4}$  Kg/cm<sup>2</sup>).

#### The Conductive Ground Plane

The conductive ground plane layer 12 may vary in thickness depending on the optical transparency and flexibility desired for the electrophotographic imaging member. For a typical flexible imaging member belt, it is desired that the thickness of the conductive ground plane 12 on the support substrate 10, for example, a titanium and/or zirconium conductive layer produced by a sputtered deposition process, is in the range of from about 2 nanometers to about 75 nanometers to effect adequate light transmission through for proper back erase. In particular embodiments, the range is from about 10 nanometers to about 20 nanometers to provide optimum combination of electrical conductivity, flexibility, and light transmission. For electrophotographic imaging process employing back exposure erase approach, a conductive ground plane light transparency of at least about 15 percent is generally desirable. The conductive ground plane need is not limited to metals. Nonetheless, the conductive ground plane 12 has usually been an electrically conductive metal layer which may be formed, for example, on the substrate by any suitable coating technique, such as a vacuum depositing or sputtering technique. Typical metals suitable for use as conductive ground plane include aluminum, zirconium, niobium, tantalum, vanadium, hafnium, titanium, nickel, stainless steel, chromium, tungsten, molybdenum, combinations thereof, and the like. Other examples of conductive ground plane 12 may be combinations of materials such as conductive indium tin oxide as a transparent layer for light having a wavelength between about 4000 Angstroms and about 9000 Angstroms or a conductive carbon black dispersed in a plastic binder as an opaque conductive layer. However, in the event where the entire substrate is chosen to be an electrically conductive metal, such as in the case that the electrophotographic imaging process designed to use front exposure erase, the outer surface thereof can perform the function of an electrically conductive ground plane so that a separate electrical conductive layer 12 may be omitted.

For the reason of convenience, all the illustrated embodiments herein after will be described in terms of a substrate layer **10** comprising an insulating material including organic polymeric materials, such as, polyethylene terephthalate (MYLAR) or polyethylene naphthalate (PEN) having a conductive ground plane **12** comprising of an electrically conductive material, such as titanium or titanium/zirconium, coating over the support substrate **10**.

#### The Hole Blocking Layer

A hole blocking layer **14** may then be applied to the conductive ground plane **12** of the support substrate **10**. Any suitable positive charge (hole) blocking layer capable of forming an effective barrier to the injection of holes from the adjacent conductive layer **12** into the overlaying photoconductive or photogenerating layer may be utilized. The charge (hole) blocking layer may include polymers, such as, polyvinylbutyral, epoxy resins, polyesters, polysiloxanes, polyamides, polyurethanes, HEMA, hydroxylpropyl cellulose, polyphosphazine, and the like, or may comprise nitrogen containing siloxanes or silanes, or nitrogen containing titanium or zirconium compounds, such as, titanate and zirconate. The hole blocking layer **14** may have a thickness in wide range of from about 5 nanometers to about 10 micrometers depending on the type of material chosen for use in a photoreceptor design. Typical hole blocking layer materials include, for example, trimethoxysilyl propylene diamine, hydrolyzed trimethoxysilyl propyl ethylene diamine, N-beta-(aminoethyl)gamma-aminopropyl trimethoxy silane, isopropyl 4-aminobenzene sulfonyl di(dodecylbenzene sulfonyl) titanate, isopropyl di(4-aminobenzoyl)isostearoyl titanate, isopropyl tri(N-ethylaminoethylamino)titanate, isopropyl tri-anthranil titanate, isopropyl tri(N,N-dimethylethylamino)titanate, titanium-4-amino benzene sulfonate oxyacetate, titanium 4-aminobenzoate isostearate oxyacetate, (gamma-aminobutyl)methyl diethoxysilane which has the formula  $[H_2N(CH_2)_4]CH_3Si(OCH_3)_2$ , and (gamma-aminopropyl) methyl diethoxysilane, which has the formula  $[H_2N(CH_2)_3]CH_3Si(OCH_3)_2$ , and combinations thereof, as disclosed, for example, in U.S. Pat. Nos. 4,338,387; 4,286,033; and 4,291,110, incorporated herein by reference in their entireties. A specific hole blocking layer comprises a reaction product between a hydrolyzed silane or mixture of hydrolyzed silanes and the oxidized surface of a metal ground plane layer. The oxidized surface forms on the outer surface of most metal ground plane layers when exposed to air after deposition. This combination enhances electrical stability at low RH. Other suitable charge blocking layer polymer compositions are also described in U.S. Pat. No. 5,244,762 which is incorporated herein by reference in its entirety. These include vinyl hydroxyl ester and vinyl hydroxy amide polymers wherein the hydroxyl groups have been partially modified to benzoate and acetate esters which modified polymers are then blended with other unmodified vinyl hydroxy ester and amide unmodified polymers. An example of such a blend is a 30 mole percent benzoate ester of poly(2-hydroxyethyl methacrylate) blended with the parent polymer poly(2-hydroxyethyl methacrylate). Still other suitable charge blocking layer polymer compositions are described in U.S. Pat. No. 4,988,597, which is incorporated herein by reference in its entirety. These include polymers containing an alkyl acrylamidoglycolate alkyl ether repeat unit. An example of such an alkyl acrylamidoglycolate alkyl ether containing polymer is the copolymer poly(methyl acrylamidoglycolate methyl ether-co-2-hydroxyethyl methacrylate). The disclosures of these U.S. patents are incorporated herein by reference in their entireties.

The hole blocking layer **14** can be continuous or substantially continuous and may have a thickness of less than about 10 micrometers because greater thicknesses may lead to undesirably high residual voltage. In aspects of the exemplary embodiment, a blocking layer of from about 0.005 micrometers to about 2 micrometers gives optimum electrical performance. The blocking layer may be applied by any suitable conventional technique, such as, spraying, dip coating, draw bar coating, gravure coating, silk screening, air knife coating, reverse roll coating, vacuum deposition, chemical treatment, and the like. For convenience in obtaining thin layers, the blocking layer may be applied in the form of a dilute solution, with the solvent being removed after deposition of the coating by conventional techniques, such as, by vacuum, heating, and the like. Generally, a weight ratio of blocking layer material and solvent of between about 0.05:100 to about 5:100 is satisfactory for spray coating.

#### The Adhesive Interface Layer

An optional separate adhesive interface layer **16** may be provided. In the embodiment illustrated in FIG. 1, an interface layer **16** is situated intermediate the blocking layer **14** and the charge generator layer **18**. The adhesive interface layer **16** may include a copolyester resin. Exemplary polyester resins which may be utilized for the interface layer include polyarylatepolyvinylbutyral, such as ARDEL POLYARYLATE (U-100) commercially available from Toyota Hsutsu Inc., VITEL PE-1200, VITEL PE-2200, VITEL PE-2200D, and VITEL PE-2222, all from Bostik, 49,000 polyester from Rohm Hass, polyvinyl butyral, and the like. The adhesive interface layer **16** may be applied directly to the hole blocking layer **14**. Thus, the adhesive interface layer **16** in embodiments is in direct contiguous contact with both the underlying hole blocking layer **14** and the overlying charge generator layer **18** to enhance adhesion bonding to provide linkage. However, in some alternative electrophotographic imaging member designs, the adhesive interface layer **16** is entirely omitted.

Any suitable solvent or solvent mixtures may be employed to form a coating solution of the polyester for the adhesive interface layer **16**. Typical solvents include tetrahydrofuran, toluene, monochlorobenzene, methylene chloride, cyclohexanone, and the like, and mixtures thereof. Any other suitable and conventional technique may be used to mix and thereafter apply the adhesive layer coating mixture to the hole blocking layer. Typical application techniques include spraying, dip coating, roll coating, wire wound rod coating, and the like. Drying of the deposited wet coating may be effected by any suitable conventional process, such as oven drying, infra red radiation drying, air drying, and the like.

The adhesive interface layer **16** may have a thickness of from about 0.01 micrometers to about 900 micrometers after drying. In embodiments, the dried thickness is from about 0.03 micrometers to about 1 micrometer.

#### The Charge Generating Layer

The photogenerating (e.g., charge generating) layer **18** may thereafter be applied to the adhesive layer **16**. Any suitable charge generating binder layer **18** including a photogenerating/photoconductive material, which may be in the form of particles and dispersed in a film forming binder, such as an inactive resin, may be utilized. Examples of photogenerating materials include, for example, inorganic photoconductive materials such as amorphous selenium, trigonal selenium, and selenium alloys selected from the group consisting of selenium-tellurium, selenium-tellurium-arsenic, selenium arsenide and mixtures thereof, and organic photoconductive materials including various phthalocyanine pigments such as the X-form of metal free phthalocyanine, metal phthalocyan-

## 11

nines such as vanadyl phthalocyanine and copper phthalocyanine, hydroxy gallium phthalocyanines, chlorogallium phthalocyanines, titanyl phthalocyanines, quinacridones, dibromo anthanthrone pigments, benzimidazole perylene, substituted 2,4-diamino-triazines, polynuclear aromatic quinones, and the like dispersed in a film forming polymeric binder. Selenium, selenium alloy, benzimidazole perylene, and the like and mixtures thereof may be formed as a continuous, homogeneous photogenerating layer. Benzimidazole perylene compositions are well known and described, for example, in U.S. Pat. No. 4,587,189, the entire disclosure thereof being incorporated herein by reference. Multi-photogenerating layer compositions may be utilized where a photoconductive layer enhances or reduces the properties of the photogenerating layer. Other suitable photogenerating materials known in the art may also be utilized, if desired. The photogenerating materials selected should be sensitive to activating radiation having a wavelength between about 400 and about 900 nm during the imagewise radiation exposure step in an electro-photographic imaging process to form an electrostatic latent image. For example, hydroxygallium phthalocyanine absorbs light of a wavelength of from about 370 to about 950 nanometers, as disclosed, for example, in U.S. Pat. No. 5,756,245.

Any suitable inactive resin materials may be employed as a binder in the photogenerating layer 18, including those described, for example, in U.S. Pat. No. 3,121,006, the entire disclosure thereof being incorporated herein by reference. Typical organic resinous binders include thermoplastic and thermosetting resins such as one or more of polycarbonates, polyesters, polyamides, polyurethanes, polystyrenes, polyarylethers, polyarylsulfones, polybutadienes, polysulfones, polyethersulfones, polyethylenes, polypropylenes, polyimides, polymethylpentenes, polyphenylene sulfides, polyvinyl butyral, polyvinyl acetate, polysiloxanes, polyacrylates, polyvinyl acetals, polyamides, polyimides, amino resins, phenylene oxide resins, terephthalic acid resins, epoxy resins, phenolic resins, polystyrene and acrylonitrile copolymers, polyvinylchloride, vinylchloride and vinyl acetate copolymers, acrylate copolymers, alkyd resins, cellulosic film formers, poly(amideimide), styrene-butadiene copolymers, vinylidenechloride/vinylchloride copolymers, vinylacetate/vinylidene chloride copolymers, styrene-alkyd resins, and the like.

An exemplary film forming polymer binder is PCZ-400 (poly(4,4'-dihydroxy-diphenyl-1-1-cyclohexane) which has a molecular weight of about 40,000 and is available from Mitsubishi Gas Chemical Corporation.

The photogenerating material can be present in the resinous binder composition in various amounts. Generally, from about 5 percent by volume to about 90 percent by volume of the photogenerating material is dispersed in about 10 percent by volume to about 95 percent by volume of the resinous binder, and more specifically from about 20 percent by volume to about 30 percent by volume of the photo generating material is dispersed in about 70 percent by volume to about 80 percent by volume of the resinous binder composition.

The photogenerating layer 18 containing the photogenerating material and the resinous binder material generally ranges in thickness of from about 0.1 micrometer to about 5 micrometers, for example, from about 0.3 micrometers to about 3 micrometers when dry. The photogenerating layer thickness is generally related to binder content. Higher binder content compositions generally employ thicker layers for photogeneration.

## The Ground Strip Layer

Other layers such as conventional ground strip layer 19 including, for example, conductive particles dispersed in a

## 12

film forming binder may be applied to one edge of the imaging member to promote electrical continuity with the conductive ground plane 12 through the hole blocking layer 14. Ground strip layer may include any suitable film forming polymer binder and electrically conductive particles. Typical ground strip materials include those enumerated in U.S. Pat. No. 4,664,995, the entire disclosure of which is incorporated by reference herein. The ground strip layer 19 may have a thickness from about 7 micrometers to about 42 micrometers, for example, from about 14 micrometers to about 23 micrometers.

## The Charge Transport Layer

The charge transport layer 20 is thereafter applied over the charge generating layer 18 and become, as shown in FIG. 1, the exposed outermost layer of the imaging member. It may include any suitable transparent organic polymer or non-polymeric material capable of supporting the injection of photogenerated holes or electrons from the charge generating layer 18 and capable of allowing the transport of these holes/electrons through the charge transport layer to selectively discharge the surface charge on the imaging member surface. In one embodiment, the charge transport layer 20 not only serves to transport holes, but also protects the charge generating layer 18 from abrasion or chemical attack and may therefore extend the service life of the imaging member. The charge transport layer 20 can be a substantially non-photocuctive material, but one which supports the injection of photogenerated holes from the charge generation layer 18. The charge transport layer 20 is normally transparent in a wavelength region in which the electro-photographic imaging member is to be used when exposure is effected therethrough to ensure that most of the incident radiation is utilized by the underlying charge generating layer 18. The charge transport layer should exhibit excellent optical transparency with negligible light absorption and neither charge generation nor discharge if any, when exposed to a wavelength of light useful in xerography, e.g., 400 to 900 nanometers. In the case when the imaging member is prepared with the use of a transparent support substrate 10 and also a transparent conductive ground plane 12, image wise exposure or erase may be accomplished through the substrate 10 with all light passing through the back side of the support substrate 10. In this particular case, the materials of the charge transport layer 20 need not have to be able to transmit light in the wavelength region of use for electro-photographic imaging processes if the charge generating layer 18 is sandwiched between the support substrate 10 and the charge transport layer 20. In all events, the exposed outermost charge transport layer 20 in conjunction with the charge generating layer 18 is an insulator to the extent that an electrostatic charge deposited/placed over the charge transport layer is not conducted in the absence of radiant illumination. Importantly, the charge transport layer 20 should trap minimal or no charges as the charge pass through it during the image copying/printing process.

The charge transport layer 20 may include any suitable charge transport component or activating compound useful as an additive molecularly dispersed in an electrically inactive polymeric material to form a solid solution and thereby making this material electrically active. The charge transport component may be added to a film forming polymeric material which is otherwise incapable of supporting the injection of photo generated holes from the generation material and incapable of allowing the transport of these holes there through. This converts the electrically inactive polymeric material to a material capable of supporting the injection of photogenerated holes from the charge generation layer 18 and capable of allowing the transport of these holes through the

charge transport layer **20** in order to discharge the surface charge on the charge transport layer. The charge transport component typically comprises small molecules of an organic compound which cooperate to transport charge between molecules and ultimately to the surface of the charge transport layer.

Any suitable inactive resin binder soluble in methylene chloride, chlorobenzene, or other suitable solvent may be employed in the charge transport layer. Exemplary binders include polyesters, polyvinyl butyral, polycarbonates, polystyrene, polyvinyl formals, and combinations thereof. The polymer binder used for the charge transport layers may be, for example, selected from the group consisting of polycarbonates, poly(vinyl carbazole), polystyrene, polyester, polyarylate, polyacrylate, polyether, polysulfone, combinations thereof, and the like. Exemplary polycarbonates include poly(4,4'-isopropylidene diphenyl carbonate), poly(4,4'-diphenyl-1,1'-cyclohexane carbonate), and combinations thereof. The molecular weight of the polymer binder used in the charge transport layer can be, for example, from about 20,000 to about 1,500,000.

Exemplary charge transport components include aromatic polyamines, such as aryl diamines and aryl triamines. Exemplary aromatic diamines include N,N'-diphenyl-N,N'-bis(alkylphenyl)-1,1'-biphenyl-4,4-diamines, such as mTBD, which has the formula (N,N'-diphenyl-N,N'-bis[3-methylphenyl]-[1,1'-biphenyl]-4,4'-diamine); N,N'-diphenyl-N,N'-bis(chlorophenyl)-1,1'-biphenyl-4,4'-diamine; and N,N'-bis-(4-methylphenyl)-N,N'-bis(4-ethylphenyl)-1,1'-3,3'-dimethylbiphenyl)-4,4'-diamine (Ae-16), N,N'-bis-(3,4-dimethylphenyl)-4,4'-biphenyl amine (Ae-18), and combinations thereof.

Other suitable charge transport components include pyrazolines, such as 1-[lepidyl-(2)]-3-(p-diethylaminophenyl)-5-(p-diethylaminophenyl)pyrazoline, as described, for example, in U.S. Pat. Nos. 4,315,982, 4,278,746, 3,837,851, and 6,214,514, substituted fluorene charge transport molecules, such as 9-(4'-dimethylaminobenzylidene)fluorene, as described in U.S. Pat. Nos. 4,245,021 and 6,214,514, oxadiazole transport molecules, such as 2,5-bis(4-diethylaminophenyl)-1,3,4-oxadiazole, pyrazoline, imidazole, triazole, as described, for example in U.S. Pat. No. 3,895,944, hydrazones, such as p-diethylaminobenzaldehyde (diphenylhydrazone), as described, for example in U.S. Pat. Nos. 4,150,987, 4,256,821, 4,297,426, 4,338,388, 4,385,106, 4,387,147, 4,399,207, 4,399,208, 6,124,514, and tri-substituted methanes, such as alkyl-bis(N,N-dialkylaminoaryl)methanes, as described, for example, in U.S. Pat. No. 3,820,989. The disclosures of all of these patents are incorporated herein by reference in their entireties.

The concentration of the charge transport component in layer **20** may be, for example, at least about 5 weight % and may comprise up to about 60 weight %. The concentration or composition of the charge transport component may vary through layer **20**, as disclosed, for example, in U.S. Pat. Nos. 7,033,714; 6,933,089; and 7,018,756, the disclosures of which are incorporated herein by reference in their entireties.

In one exemplary embodiment, charge transport layer **20** comprises an average of about 10 to about 60 weight percent N,N'-diphenyl-N,N'-bis(3-methylphenyl)-1,1'-biphenyl-4,4'-diamine, or from about 30 to about 50 weight percent N,N'-diphenyl-N,N'-bis(3-methylphenyl)-1,1'-biphenyl-4,4'-diamine.

The charge transport layer **20** is an insulator to the extent that the electrostatic charge placed on the charge transport layer is not conducted in the absence of illumination at a rate sufficient to prevent formation and retention of an electro-

static latent image thereon. In general, the ratio of the thickness of the charge transport layer **20** to the charge generator layer **18** is maintained from about 2:1 to about 200:1 and in some instances as great as about 400:1.

Additional aspects relate to the inclusion in the charge transport layer **20** of variable amounts of an antioxidant, such as a hindered phenol. Exemplary hindered phenols include octadecyl-3,5-di-tert-butyl-4-hydroxyhydrocinnamate, available as IRGANOX 1-1010 from Ciba Specialty Chemicals. The hindered phenol may be present at about 10 weight percent based on the concentration of the charge transport component. Other suitable antioxidants are described, for example, in above-mentioned U.S. Pat. No. 7,018,756 incorporated by reference.

In one specific embodiment, the charge transport layer **20** is a solid solution including a charge transport component, such as N,N'-diphenyl-N,N'-bis(3-methylphenyl)-1,1'-biphenyl-4,4'-diamine, molecularly dissolved in a polycarbonate binder, the binder being either a bisphenol A polycarbonate of poly(4,4'-isopropylidene diphenyl carbonate) or a bisphenol Z polycarbonate of poly(4,4'-diphenyl-1,1'-cyclohexane carbonate). The bisphenol A polycarbonate used for typical charge transport layer formulation is FPC 0170, having a molecular weight of about 120,000 and commercially available from Mitsubishi Chemicals Corp. The molecular structure of bisphenol A polycarbonate, poly(4,4'-isopropylidene diphenyl carbonate), is given in Formula (A) below:



wherein n indicates the degree of polymerization. In the alternative, poly(4,4'-diphenyl-1,1'-cyclohexane carbonate) may also be used to for the anticurl back coating in place of FPC 0170 bisphenol A polycarbonate. The molecular structure of poly(4,4'-diphenyl-1,1'-cyclohexane carbonate), having a weight average molecular weight of about between about 20,000 and about 200,000, is given in Formula (B) below:



wherein n indicates the degree of polymerization.

The charge transport layer **20** may have between about 10 and about 50 micrometers in thickness, or between about 20 and about 40 micrometers. The typical charge transport layer has a Young's Modulus in the range of from about  $2.5 \times 10^{-5}$  psi ( $1.7 \times 10^{-4}$  Kg/cm<sup>2</sup>) to about  $4.5 \times 10^{-5}$  psi ( $3.2 \times 10^{-4}$  Kg/cm<sup>2</sup>) and a thermal contraction coefficient of between about  $6 \times 10^{-5}$  °C. and about  $8 \times 10^{-5}$  °C. Since the charge transport layer **20** does have a substantially greater thermal contraction coefficient constant compared to that of the support substrate **10**, the prepared flexible electrophotographic imaging member (using a 3-mil flexible biaxially oriented PET substrate and a 25 micrometers charge transport layer)

will exhibit spontaneous upward curling, into a 1½ inch roll if unrestrained, due to the result of larger dimensional contraction in the charge transport layer **20** than the support substrate **10**, as the imaging member cools from the glass transition temperature of the charge transport layer down to room ambient temperature of 25° C. after the heating/drying processes of the applied wet charge transport layer coating. The consequence of greater dimensional contraction of the charge transport layer **20** than that of the substrate support **10** after cooling causes internal tension build-up in the layer to pull the imaging member inwardly and result in imaging member curling.

An anti-curl back coating **1** is therefore need and applied to the back side of the support substrate **10** (which is the side opposite the side bearing the electrically active coating layers) in order to render the prepared imaging member with desired flatness.

#### The Anticurl Back Coating

Since the charge transport layer **20** is applied by solution coating process, the applied wet film is dried at elevated temperature and then subsequently cooled down to room ambient. The resulting imaging member web (comprising a 25 micrometers charge transport layer and a 3 mils PET substrate) if, at this point, not restrained, will spontaneously curl upwardly into a 1½ inch tube due to greater dimensional contraction and shrinkage of the Charge transport layer than that of the substrate support layer **10**. An anti-curl back coating **1**, as the conventional imaging member shown in FIG. 1, is then applied to the back side of the support substrate **10** (which is the side opposite the side bearing the electrically active coating layers) in order to render the prepared imaging member with desired flatness.

Generally, the anticurl back coating **1** comprises a thermoplastic polymer and an adhesion promoter. The thermoplastic polymer, in some embodiments being the same as the polymer binder used in the charge transport layer, is typically a bisphenol A polycarbonate, which along with the addition of an adhesion promoter of polyester are both dissolved in a solvent to form an anticurl back coating solution. The coated anticurl back coating **1** must adhere well to the support substrate **10** to prevent premature layer delamination during imaging member belt machine function in the field.

In a conventional anticurl back coating, an adhesion promoter of copolyester is included in the bisphenol A polycarbonate poly(4,4'-isopropylidene diphenyl carbonate) material matrix to provide adhesion bonding enhancement to the substrate support. Satisfactory adhesion promoter content is from about 0.2 percent to about 20 percent or from about 2 percent to about 10 percent by weight, based on the total weight of the anticurl back coating. The adhesion promoter may be any known in the art, such as for example, VITEL PE2200 which is available from Bostik, Inc. (Middleton, Mass.). The anticurl back coating has a thickness that is adequate to counteract the imaging member upward curling and provide flatness. In embodiments, the anticurl back coat-

ing has a thickness of from about 5 to about 40 micrometers or between about 10 and about 20 micrometers. A typical, conventional anticurl back coating formulation is a 92:8 ratio of polycarbonate to adhesive.

FIG. 2 discloses a flexible imaging member prepared according to the material formulation and methodology of the present disclosure to have an amine species resistance charge transport layer formulation. In the embodiments, the substrate **10**, conductive ground plane **12**, hole blocking layer, **14**, adhesive interface layer **16**, charge generating layer **18**, ground strip layer **16**, charge transport layer **20**, and anticurl back coating **1** of the disclosed imaging member are prepared to include the same materials, compositions, thicknesses, and follow the identical procedures as those described in the conventional imaging member of FIG. 1, but with the exception that the charge transport layer **20** is reformulated to use a novel A-B diblock copolymer binder **24** of this disclosure.

According to aspects illustrated herein, there is provided a flexible imaging member comprising a flexible substrate **10**, a conductive ground plane **12**, a hole blocking layer, **14**, an adhesive interface layer **16**, a charge generating layer **18** disposed on the adhesive interface layer **16**, a ground strip layer **16**, and a charge transport layer **20** of present disclosure disposed on the charge generating layer **18**, and an anticurl back coating **1** to maintain imaging member flatness. The disclosed charge transport layer **20** is a binary solid solution formulated to comprise a charge transport compound of N,N'-diphenyl-N,N'-bis(3-methylphenyl)-1,1-biphenyl-4,4'-diamine molecularly dispersed a novel copolymer binder **24**. The novel copolymer binder **24** is a film forming A-B diblock copolymer which is created by modifying the bisphenol A polycarbonate poly(4,4'-isopropylidene diphenyl carbonate) to include a phthalic acid containing segmental block at the terminal of the bisphenol A polycarbonate back bone. The charge transport compound N,N'-diphenyl-N,N'-bis(3-methylphenyl)-1,1-biphenyl-4,4'-diamine presence in the disclosed charge transport layer **20** is from about 20 to about 80 weight percent, or from about 30 to about 60 weight percent, based on the total weight of the charge transport layer, for effecting optimum photo-electrical and mechanical performances. The resulting charge transport layer **20** thus prepared has a thickness of from about 20 to about 40 micrometers.

In the example of one specific electrophotographic imaging member, the charge transport layer **20** of the present disclosure is formulated to comprise a charge transport component molecularly dispersed in the novel film forming A-B diblock copolymer binder; the copolymer binder is created by modifying the bisphenol A polycarbonate poly(4,4'-isopropylidene diphenyl carbonate) to include a phthalic acid containing segmental block at the terminal of bisphenol A polycarbonate back bone. So, the A-B di-block copolymer is consisting of a bisphenol A polycarbonate segment block A which is linking to a phthalic acid containing segment block B, having a general molecular structure shown in Formula (I) below:



In another electrophotographic imaging member example, the disclosed charge transport layer **20** is also formulated to comprise a charge transport component molecularly dispersed in a likewise film forming A-B diblock copolymer binder **24** consisting of bisphenol A polycarbonate poly(4,4'-isopropylidene diphenyl carbonate) block A and a phthalic acid containing segmental block B at the terminal of bisphenol A polycarbonate back bone. The likewise A-B di-block copolymer of the bisphenol A polycarbonate does have a general molecular structure shown in the following Formula (II):

sized here, is the capability of the phthalic acid terminal to provide amine species quenching/neutralization effect for absolute elimination of the root cause of copy ghosting defects printout problem.

In the extended embodiments of this disclosure shown in FIG. 2, the bisphenol A segmental block (A) of the film forming A-B di-block copolymer of Formulas (I) and (II) used for charge transport layer formulation may alternatively include each of the other types of bisphenol carbonates selected to consist of:



In the above formulas, z represents the number of bisphenol A repeating units in block A of from about 9 to about 18, y is number of repeating phthalic acid block B of from about 1 to about 2, and n is the degree of polymerization. The degree of polymerization, n, is between about 20 and about 80 of the diblock copolymer having molecular weight between about 100,000 and about 200,000.

The film forming A-B diblock copolymer **24**, derived and modified from a bisphenol A polycarbonate, is a creation of the bisphenol A polycarbonate to include small fraction of phthalic acid such that the resulting copolymer contains about 90 mole percent of a bisphenol A segment block A linearly linking to about 10 mole percent of a segmental block B of phthalic acid terminal in the A-B diblock copolymer chain. The phthalic acid terminal in the A-B diblock copolymer molecule of both Formulas (I) and (II) may either be a terephthalic acid or an isophthalic acid represented by the following, respectively:



The specific A-B diblock copolymer chosen to meet the present flexible imaging member charge transport layer disclosure formulation requirement is LEXAN HLX polymer available from Sabic Innovative Plastics (Pittsfield, Mass.). Since the LEXAN HLX (as described in the above Formulas (I) and (II)) is a film forming polycarbonate/phthalic acid copolymer and has the physical/mechanical/thermal properties equivalent to those of the conventional polycarbonate counterpart used as charge transport layer binder in prior art imaging members, so utilization of it for charge transport layer disclosure formulation is a direct and simple approach. The key benefit of choosing LEXAN HLX polymer for charge transport layer **20** binder application, to be emphasized



The phthalic acid containing block B linkage is selected from one consisting of the groups:



19



Additionally, the block (B) phthalic acid containing terminal in the A-B diblock copolymers (having all the alternative structures described above) may be a terephthalic acid or an isophthalic acid represented by the following, respectively:



Furthermore, the phthalic acid terminal may alternatively be replaced with an adipic acid or an azelaic acid shown by the following, respectively:



In the further extended embodiments of flexible imaging member disclosure, shown in FIG. 3, the charge transport layer **20** of FIG. 2 is then redesigned to consist of dual layers: a bottom layer **20B** and a top exposed layer **20T**. Both of these layers comprise about the same thickness and utilizing the same A-B diblock copolymer binder **24** and same charge transport compound of N,N'-diphenyl-N,N'-bis(3-methylphenyl)-1,1-biphenyl-4,4'-diamine, with the bottom layer contains a greater amount of the charge transport compound than that in the top exposed layer. The charge transport compound presence in the bottom layer **20B** is between about 60 and about 80 weight percent while that in the top exposed layer **20T** is between about 40 and about 20 weight percent based on the total weight of each respective layer to impact optimum photo-electrical and mechanical functions. The both disclosed dual charge transport layers are of the same thickness and have a total thickness of between about 20 and about 40 micrometers.

In yet further extended embodiments of flexible imaging member of the present disclosure, wherein the charge transport layer is re-formulated to have triple charge transport

20

layers consisting of bottom layer **20B**, center layer **20C**, and top exposed layer **20T** as illustrated in FIG. 4. All the triple layers comprise about the same thickness and utilizing the same A-B diblock copolymer binder **24** as well as same charge transport compound of N,N'-diphenyl-N,N'-bis(3-methylphenyl)-1,1-biphenyl-4,4'-diamine, with the bottom layer **20B** contains the greatest and the top exposed layer **20T** the least amount of the charge transport compound. The charge transport compound presence in the bottom layer **20B** is from about 70 to about 90 weight percent, that in the center layer **20C** is from about 40 to about 60 weight percent, and that in the top exposed layer **20T** is from about 20 to about 30 weight percent based on the total weight of each respective layer. The disclosed triple charge transport layers are of the same thickness and have a total thickness of from about 20 to about 40 micrometers.

In still yet further extended embodiments of flexible imaging member of this disclosure, the charge transport layer is further re-formulated to have multiple charge transport layers consisting of first/bottom layer **20F**, middle plurality of layers **20M**, and last/top exposed layer **20L** as shown in FIG. 5. All these charge transport layers comprise about the same thickness and utilizing the same A-B diblock copolymer binder **24** as well as same charge transport compound of N,N'-diphenyl-N,N'-bis(3-methylphenyl)-1,1-biphenyl-4,4'-diamine, but with the exception that the amount of charge transport compound in each layer is decreased in continuum starting from the first/bottom layer **20F** reaches toward the last/top outermost exposed layer **20L** of the imaging member, so that the lowest amount is present in the last outermost exposed layer. That means the content of the A-B diblock copolymer binder **24** counterpart in each layer is vice versa increased, starting from the lowest in first/bottom layer **20F** rises continuously toward the top such that the last/top outermost layer **20L** has the highest content of copolymer binder **24**. From optimum photo-electrical and mechanical function consideration, the charge transport compound presence in the first/bottom layer **20F** is from about 70 to about 90 weight percent while that in the last/top exposed layer **20L** is from about 20 to about 30 weight percent based on the total weight of each respective layer.

In the embodiments where the charge transport layer comprises multiple layers, with reference to FIG. 5, the layers may have a total of from about 4 to about 10 discreet layers, or from about 4 to about 6. While the thickness of each of the charge transport layers **20F**, **20M**, and **40L** may be different, but they are preferably to be the same and range from about 0.5 to about 7 micrometers. Generally, the disclosed multiple charge transport layers have a total thickness of between about 20 and about 40 micrometers.

As an alternative to the two discretely separated layers of being a charge transport **20** and a charge generation layers **18** as those described in FIG. 1, a structurally simplified imaging member, having all other layers being formed in the same manners as described in preceding figures, may be created to contain a single imaging layer **22** having both charge generating and charge transporting capabilities and with the use of the novel A-B diblock copolymer binder **24** as illustration shown in FIG. 6. In a prior art electrophotographic imaging member design, the single imaging layer **22** comprises a single electrophotographically active layer capable of retaining an electrostatic charge in the dark during electrostatic charging, imagewise exposure and image development, as disclosed, for example, in U.S. Pat. No. 6,756,169. The single imaging layer **22** is to be formed to include charge transport molecules in a binder the novel A-B diblock copolymer binder **24** of this disclosure, the same to those of the charge

transport layer **20** previously described in FIG. 1, and may also optionally include a photogenerating/photoconductive material similar to those of the layer **18** as described. In exemplary embodiments, the single imaging layer **22** of the flexible imaging member of the present disclosure, shown in FIG. 6, is formulated to comprise a charge transport compound, a photogenerating/photoconductive material, and the A-B diblock copolymer **24**.

The flexible imaging members of present disclosure, is prepared to contain an acid containing A-B diblock copolymer binder **24** in the charge transport layer(s) for active quenching/neutralization the amine species and resolve the ghosting defects issue in the print out copy. The resulting imaging members thus obtained do have enhanced mechanical function as well as preserved the photoelectrical integrity with respect to each control imaging member. That means, for example, having charge acceptance ( $V_o$ ) in a range of from about 750 to about 850 volts; sensitivity (S) sensitivity from about 250 to about 450 volts/ergs/cm<sup>2</sup>; residual potential ( $V_r$ ) less than about 100 volts; an a depletion potential ( $V_{depl}$ ) of less than 200 volts.

The resulting charge transport layer prepared according to the description of present disclosure (only the top exposed layer of the multiple layers) may also contain a light shock resisting or reducing agent of from about 1 to about 6 wt-%. Such light shock resisting agents include 3,3',5,5'-tetra(t-butyl)-4,4'-diphenoxquinone (DPQ); 5,6,11,12-tetraphenyl naphthacene (Rubrene); 2,2'-[cyclohexylidenebis[(2-methyl-4,1-phenylene)azo]]bis[4-cyclohexyl-(9Cl)]; perinones; perylenes; and dibromo anthanthrone (DBA). To further improved the disclosed imaging member's dmechanical performance, top charge transport layer, being a single layer or multiple layers, may also include the additive of inorganic or organic fillers to impart greater wear resistant enhancement. Inorganic fillers may include, but are not limited to, silica, metal oxides, metal carbonate, metal silicates, and the like. Examples of organic fillers include, but are not limited to, KEVLAR, stearates, fluorocarbon (PTFE) polymers such as POLYMIST and ZONYL, waxy polyethylene such as ACUMIST and ACRAWAX, fatty amides such as PETRAC erucamide, oleamide, and stearamide, and the like. Either micron-sized or nano-sized inorganic or organic particles can be used in the fillers to achieve mechanical property reinforcement. One suitable particulate dispersion is described in U.S. Pat. No. 6,326,111, which is hereby incorporated by reference in its entirety.

For typical conventional ionographic imaging members preparation used in an electrographic system, the dielectric layer overlying the conductive layer of a substrate may also use the novel A-B diblock copolymer of this disclosure to replace all the active photoconductive layers. If required, the flexible electrographic belts may also comprise an ACBC to provide belt flatness.

The flexible multilayered electrophotographic imaging member fabricated in accordance with the embodiments of present disclosure, described in all the above preceding, may be cut into rectangular sheets. A pair of opposite ends of each imaging member cut sheet is then brought overlapped together thereof and joined by any suitable means, such as ultrasonic welding, gluing, taping, stapling, or pressure and heat fusing to form a continuous imaging member seamed belt, sleeve, or cylinder.

A prepared flexible imaging belt thus may thereafter be employed in any suitable and conventional electrophotographic imaging process which utilizes uniform charging prior to imagewise exposure to activating electromagnetic radiation. When the imaging surface of an electrophoto-

graphic member is uniformly charged with an electrostatic charge and imagewise exposed to activating electromagnetic radiation, conventional positive or reversal development techniques may be employed to form a marking material image on the imaging surface of the electrophotographic imaging member. Thus, by applying a suitable electrical bias and selecting toner having the appropriate polarity of electrical charge, a toner image is formed in the charged areas or discharged areas on the imaging surface of the electrophotographic imaging member. For example, for positive development, charged toner particles are attracted to the oppositely charged electrostatic areas of the imaging surface and for reversal development, charged toner particles are attracted to the discharged areas of the imaging surface.

Furthermore, a prepared electrophotographic imaging member belt can additionally be evaluated by printing in a marking engine into which the belt, formed according to the exemplary embodiments, has been installed. For intrinsic electrical properties it can also be determined by conventional electrical drum scanners. Additionally, the assessment of its propensity of developing streak line defects print out in copies can alternatively be carried out by using electrical analyzing techniques, such as those disclosed in U.S. Pat. Nos. 5,703,487; 5,697,024; 6,008,653; 6,119,536; and 6,150,824, which are incorporated herein in their entireties by reference. All the patents and applications referred to herein are hereby specifically, and totally incorporated herein by reference in their entirety in the instant specification.

All the exemplary embodiments encompassed herein include a method of imaging which includes generating an electrostatic latent image on an imaging member, developing a latent image, and transferring the developed electrostatic image to a suitable substrate.

While the description above refers to particular embodiments, it will be understood that many modifications may be made without departing from the spirit thereof. The accompanying claims are intended to cover such modifications as would fall within the true scope and spirit of embodiments herein.

## EXAMPLES

The development of the presently disclosed embodiments will further be demonstrated in the non-limiting working examples below. They are, therefore in all respects, to be considered as illustrative and not restrictive nor limited to the materials, conditions, process parameters, and the like recited herein. The scope of embodiments are being indicated by the appended claims rather than the foregoing description. All changes that come within the meaning of and range of equivalency of the claims are intended to be embraced therein. All proportions are by weight unless otherwise indicated. It will be apparent, however, that the present embodiments can be practiced with many types of compositions and can have many different uses in accordance with the disclosure above and as pointed out hereinafter.

### Control Example

A conventional prior art flexible electrophotographic imaging member web, as shown in FIG. 1, was prepared by providing a 0.02 micrometer thick titanium layer **12** coated substrate of a biaxially oriented polyethylene naphthalate substrate **10** (PEN, available as KADALEX from DuPont Teijin Films.) having a thickness of 3.5 mils. The titanized KADALEX substrate was extrusion coated with a blocking layer solution containing a mixture of 6.5 grams of gamma

aminopropyltriethoxy silane, 39.4 grams of distilled water, 2.08 grams of acetic acid, 752.2 grams of 200 proof denatured alcohol and 200 grams of heptane. This wet coating layer was then allowed to dry for 5 minutes at 135° C. in a forced air oven to remove the solvents from the coating and effect the formation of a crosslinked silane blocking layer. The resulting blocking layer 14 had an average dry thickness of 0.04 micrometer as measured with an ellipsometer.

An adhesive interface layer 16 was then applied by extrusion coating to the blocking layer with a coating solution containing 0.16 percent by weight of ARDEL polyarylate, having a weight average molecular weight of about 54,000, available from Toyota Hsushu, Inc., based on the total weight of the solution in an 8:1:1 weight ratio of tetrahydrofuran/monochloro-benzene/methylene chloride solvent mixture. The adhesive interface layer was allowed to dry for 1 minute at 125° C. in a forced air oven. The resulting adhesive interface layer 16 had a dry thickness of about 0.02 micrometer.

The adhesive interface layer was thereafter coated over with a charge generating layer 18. The charge generating layer dispersion was prepared by adding 0.45 gram of IUPILON 200, a polycarbonate of poly(4,4'-diphenyl)-1,1'-cyclohexane carbonate (PCZ 200, available from Mitsubishi Gas Chemical Corporation), and 50 milliliters of tetrahydrofuran into a 4 ounce glass bottle. 2.4 grams of hydroxygallium phthalocyanine Type V and 300 grams of 1/8 inch (3.2 millimeters) diameter stainless steel shot were added to the solution. This mixture was then placed on a ball mill for about 20 to about 24 hours. Subsequently, 2.25 grams of poly(4,4'-diphenyl-1,1'-cyclohexane carbonate) having a weight average molecular weight of 20,000 (PC-Z 200) were dissolved in 46.1 grams of tetrahydrofuran, then added to the hydroxygallium phthalocyanine slurry. This slurry was then placed on a shaker for 10 minutes. The resulting slurry was thereafter coated onto the adhesive interface by extrusion application process to form a layer having a wet thickness of 0.25 mil. However, a strip of about 10 millimeters wide along one edge of the substrate web stock bearing the blocking layer and the adhesive layer was deliberately left uncoated by the charge generating layer (CGL) to facilitate adequate electrical contact by a ground strip layer 19 to be applied later. This CGL comprised of poly(4,4'-diphenyl)-1,1'-cyclohexane carbonate, tetrahydrofuran and hydroxygallium phthalocyanine was dried at 125° C. for 2 minutes in a forced air oven to form a dry charge generating layer 18 having a thickness of 0.7 micrometers.

This coated web was simultaneously coated over with a charge transport layer 20 and a ground strip layer 19 by co-extrusion of the coating materials. The charge transport layer was prepared by introducing into an amber glass bottle in a weight ratio of 1:1 (or 50 weight percent of each) of a bisphenol A polycarbonate thermoplastic (FPC 0170, having a molecular weight of about 120,000 and commercially available from Mitsubishi Chemicals Corp.) and a diamine charge transport compound of N,N'-diphenyl-N,N'-bis(3-methylphenyl)-1,1'-biphenyl-4,4'-diamine.

The resulting mixture was dissolved to give 15 percent by weight solid in methylene chloride. This solution was applied on the CGL 18 by extrusion process to form a coating which after drying in a forced air oven gave a 29 micrometers thick dry charge transport layer (CTL) 20 comprising 50:50 weight ratio of diamine transport charge transport compound to FPC0170 bisphenol A polycarbonate binder. The imaging member web, at this point if unrestrained, would curl upwardly into a 1 3/4-inch tube.

The strip, about 10 millimeters wide, of the adhesive layer left uncoated by the CGL, was coated with a ground strip

layer during the co-extrusion process. The ground strip layer coating mixture was prepared by combining 23.81 grams of polycarbonate resin (FPC 0170, available from Mitsubishi Chemical Corp.) having 7.87 percent by total weight solids and 332 grams of methylene chloride in a carboy container. The container was covered tightly and placed on a roll mill for about 24 hours until the polycarbonate was dissolved in the methylene chloride. The resulting solution was mixed for 15-30 minutes with about 93.89 grams of graphite dispersion (12.3 percent by weight solids) of 9.41 parts by weight of graphite, 2.87 parts by weight of ethyl cellulose and 87.7 parts by weight of solvent (ACHESON Graphite dispersion RW22790, available from Acheson Colloids Company (Port Huron, Mich.)) with the aid of a high shear blade dispersed in a water cooled, jacketed container to prevent the dispersion from overheating and losing solvent. The resulting dispersion was then filtered and the viscosity was adjusted with the aid of methylene chloride. This ground strip layer coating mixture was then applied, by co-extrusion with the CTL, to the electrophotographic imaging member web to form an electrically conductive ground strip layer.

The imaging member web stock containing all of the above layers was then transported at 60 feet per minute web speed and passed through 125° C. production coater forced air oven to dry the co-extrusion coated ground strip 16 and CTL 20 simultaneously to give respective 19 micrometers and 29 micrometers in dried thicknesses after eventual cooling down to room ambient. The resulting imaging member web had a 29 micrometer-thick single layered CTL 20, according to the conventional art shown in FIG. 1, but without application of an anticurl back coating was seen, if unrestrained as it cooled down to room ambient of 25° C., to spontaneously curl upwardly into a 1 1/2 inch roll. The prepared imaging member web was to be used to serve as a control.

An anticurl back coating was prepared by combining 882 grams of FPC 0170 polycarbonate resin ( ), 71.2 grams VITEL PE-200 copolyester (available from Goodyear Tire and Rubber Company) and 10,710 grams of methylene chloride in a carboy container to form a coating solution containing 8.9 percent solids. The container was covered tightly and placed on a roll mill for about 24 hours until the polycarbonate and polyester were dissolved in the methylene chloride to form the anti-curl back coating solution. The anticurl back coating solution was then applied to the rear surface (side opposite the charge generating layer and charge transport layer) of the electrophotographic imaging member web by extrusion coating and dried to a maximum temperature of 125° C. through the forced air oven to produce a dried coating layer having a thickness of 17 micrometers and render the imaging member web with desirable flatness

#### Disclosure Example

A flexible electrophotographic imaging member web, as shown in FIG. 2, was prepared with the exact same material compositions as the Control Example and following identical procedures as those described in the Control Example, but with the exception that FPC 0170 polycarbonate binder in the single charge transport layer 20 of the imaging member web was totally replaced with a novel A-B diblock copolymer 24. The A-B di-block copolymer 24 (LEXAN HLX polycarbonate, available from Sabic Innovative Plastics) is consisting of 90 mole percent of bisphenol A polycarbonate segment block A which is linking to 10 mole percent of phthalic acid containing segment block B. LEXAN HLX polycarbonate as received has a molecular weight of about 115,000 and is a mixture of the two general molecular structures shown in Formulas (I) and (II) below:



wherein z representing the numbers of bisphenol A repeating units of block A has a value of 9; y of 1 is the number of repeating phthalic acid unit of block B; and n is the degree of polymerization of the A-B diblock copolymer having a molecular weight of about 115,000, as available from Sabic Innovative Plastics.

Physical/Mechanical and Photoelectrical Measurements

The photoelectrical properties of the imaging member webs of the Control and the Disclosure Examples were determined by using the 4000 scanner. The measurement results thus obtained (shown in Table 1 below) indicate that the disclosed imaging member prepared to employ a binder of phthalic acid terminated A-B diblock copolymer of bisphenol A polycarbonate in the charge transport layer 20, for effecting amine compound elimination/neutralization, did not cause any adverse impact to photoelectrical integrity of the original imaging member control. In conclusion, the disclosure imaging member having the charge transport layer 20 reformulated by using the phthalic acid containing bisphenol A polycarbonate binder for total FPC 0170 polycarbonate replacement should therefore provide effective suppression/elimination of the current pre-printed paper ghosting defects copy printout problem. Furthermore, having a molecular weight of about 115,000, the reformulated charge transport (CTL) 20 layer of this disclosure should maintain the mechanical function integrity equivalent to that of the of the control counterpart.

It will be appreciated that several of the above-disclosed and other features and functions, or alternatives thereof, may be desirably combined into many other different systems or applications. Also that various presently unforeseen or unanticipated alternatives, modifications, variations or improvements therein may be subsequently made by those skilled in the art which are also intended to be encompassed by the following claims. Unless specifically recited in a claim, steps or components of claims should not be implied or imported from the specification or any other claims as to any particular order, number, position, size, shape, angle, color, or material.

What is claimed is:

1. An imaging member comprising:  
a flexible substrate;  
a charge generating layer disposed on the substrate; and  
at least one charge transport layer disposed on the charge generating layer, wherein the charge transport layer comprises a charge transport component molecularly dispersed in a polycarbonate binder, the polycarbonate binder being an A-B diblock copolymer comprising two segmental blocks of a bisphenol A polycarbonate ( $C_{16}H_{14}O_3$ ) and a phthalic acid capable of providing protection against amine species contaminants; wherein the diblock copolymer binder in the at least one charge transport layer has a formula selected from the group consisting of

| TABLE 1          |                |     |     |     |      |             |       |
|------------------|----------------|-----|-----|-----|------|-------------|-------|
| Sample ID        | CTL Binder     | Vo  | S   | Vc  | Vr   | $V_{e-6.0}$ | Vdepl |
| Control          | Poly-carbonate | 799 | 351 | 160 | 26.5 | 44.9        | 56.2  |
| Disclosure       | LEXAN HLX      | 799 | 334 | 165 | 26.9 | 47.9        | 53.9  |
| After 10K cycles |                |     |     |     |      |             |       |
| Control          | Poly-carbonate | 799 | 333 | 194 | 45.9 | 74.4        | 104.8 |
| Disclosure       | LEXAN HLX      | 799 | 326 | 182 | 33   | 59.5        | 105.1 |
|                  |                |     |     |     |      |             | -54.3 |

All the patents and applications referred to herein are hereby specifically, and totally incorporated herein by reference in their entirety in the instant specification.



wherein z representing the number of bisphenol A repeating units in block A is from about 9 to about 18, y representing the number of repeating phthalic acid in block B is from about 1 to about 2, and n representing the degree of polymerization of diblock copolymer is from about 20 to about 80; and mixtures thereof.

2. The imaging member of claim 1, wherein the copolymer binder has a molecular weight of from about 100,000 to about 200,000.

3. The imaging member of claim 1, wherein the charge transport component is N,N'-diphenyl-N,N'-bis(3-methylphenyl)-1,1-biphenyl-4,4'-diamine.

4. The imaging member of claim 1, wherein the charge transport component present in the charge transport layer is from about 20 to about 80 weight percent based on the total weight of the charge transport compound and the diblock copolymer binder in the layer.

5. The imaging member of claim 1, wherein the thickness of the at least one charge transport layer is from about 20 micrometers to about 40 micrometers.

6. The imaging member of claim 1, wherein the charge transport layer is a dual-layer including a bottom charge transport layer and a top exposed charge transport layer disposed on the bottom charge transport layer, and further wherein both the bottom and the top exposed charge transport layers have the same thickness with a total thickness of from about 20 to about 40 micrometers.

7. The imaging member of claim 6, wherein the charge transport component present in the bottom charge transport layer in an amount of from about 60 to about 80 weight percent and is present in the top exposed charge transport layer in an amount of from about 20 to about 40 weight percent, based on the total weight of the charge transport compound and the diblock copolymer binder in each respective layer.

8. The imaging member of claim 1, wherein the charge transport layer is a triple-layer including a bottom charge transport layer, a center charge transport layer disposed on the bottom charge transport layer, and a top exposed charge trans-

layers disposed on the bottom charge transport layer, and a top exposed charge transport layer disposed on the plurality of middle charge transport layers.

11. The imaging member of claim 10, wherein the multiple charge transport layers comprises from about 4 to about 15 charge transport layers or from about 4 to about 6 charge transport layers, and further wherein each of the multiple charge transport layers have the same thickness with a total thickness of from 20 to about 40 micrometers.

12. The imaging member of claim 11, wherein the amount of charge transport component present in the multiple charge transport layers decreases in continuum from the bottom charge transport layer to the top exposed charge transport layer.

13. The imaging member of claim 12, wherein the charge transport component is present in the bottom charge transport layer in an amount of from about 70 to about 90 weight percent and is present in the top exposed charge transport layer in an amount of from about 20 to about 30 weight percent based on the total weight of the charge transport compound and the diblock copolymer binder in each respective layer.

14. The imaging member of claim 1, wherein the phthalic acid in the segmental block (B) is selected from the group consisting of terephthalic acid, isophthalic acid, adipic acid, azelaic acid, and mixtures thereof.

15. An imaging member comprising:  
a substrate;  
a charge generating layer disposed on the substrate;  
a bottom charge transport layer disposed on the charge generating layer; and a top exposed charge transport layer disposed on the bottom charge transport layer, wherein both the bottom and the top exposed charge transport layers comprise N,N'-diphenyl-N,N'-bis(3-methylphenyl)-1,1-biphenyl-4,4'-diamine molecularly dispersed in a polycarbonate binder, the polycarbonate binder having a formula selected from the group consisting of



port layer disposed on the center charge transport layer, and further wherein each of the three charge transport layers have the same thickness with a total thickness of from about 20 to about 40 micrometers.

9. The imaging member of claim 8, wherein the charge transport component is present in the bottom charge transport layer in an amount of from about 70 to about 90 weight percent, is present in the center charge transport layer in an amount of from about 40 to about 60 weight percent, and is present in the top exposed charge transport layer in an amount of from about 20 to about 30 weight percent based on the total weight of the charge transport compound and the diblock copolymer binder in each respective layer.

10. The imaging member of claim 1, wherein the charge transport layer comprises multiple layers including a bottom charge transport layer, a plurality of middle charge transport

wherein z represents the number of bisphenol A repeating units in block A and is from about 9 to about 18, y represents the number of repeating phthalic acid in block B and is from about 1 to about 2, and n represents the degree of polymerization of di-block copolymer and is from about 20 to about 80 for the diblock copolymer having a molecular weight of from about 100,000 to about 200,000.

16. The imaging member of claim 15, wherein the bottom and the top exposed charge transport layers have the same thickness with a total thickness of from about 20 to about 40 micrometers.

17. The imaging member of claim 15, wherein an amount of the charge transport component present in the bottom charge transport layer is greater than that present in the top exposed charge transport layer.

29

18. The imaging member of claim 17, wherein an amount of the charge transport component present in the bottom charge transport layer is from about 60 to about 80 weight percent and an amount of the charge transport component in the top exposed charge transport layer is from about 20 to about 40 weight percent based on the total weight of the charge transport compound and the diblock copolymer binder in each respective layer.

19. An image forming apparatus for forming images on a recording medium comprising:

- a) an imaging member having a charge retentive-surface for receiving an electrostatic latent image thereon, wherein the imaging member comprises

5

10

30

a flexible substrate; a charge generating layer disposed on the substrate; and at least one charge transport layer disposed on the charge generating layer, wherein the charge transport layer comprises a charge transport component molecularly dispersed in a polycarbonate binder, the polycarbonate binder being an A-B di-block copolymer comprising two segmental blocks of a Bisphenol A polycarbonate ( $C_{16}H_{14}O_3$ ) and a phthalic acid; wherein the diblock copolymer binder in the at least one charge transport layer has a formula selected from the group consisting of



25

30

35

wherein z representing the number of bisphenol A repeating units in block A is from about 9 to about 18, y representing the number of repeating phthalic acid in block B is from about 1 to about 2, and n representing the degree of polymerization of diblock copolymer is from about 20 to about 80; and mixtures thereof;

b) a development component for applying a developer material to the charge-retentive surface to develop the electrostatic latent image to form a developed image on the charge-retentive surface;

c) a transfer component for transferring the developed image from the charge-retentive surface to a copy substrate; and

d) a fusing component for fusing the developed image to the copy substrate.

\* \* \* \* \*